

June 8, 1926.

1,587,697

A. L. CLAPP

HEEL FOR WOMEN'S SHOES AND METHOD OF MAKING

Filed March 7, 1924



Inventor:  
Albert L. Clapp,  
by right from him by May  
27, 1925.

Patented June 8, 1926.

1,587,697

# UNITED STATES PATENT OFFICE.

ALBERT L. CLAPP, OF DANVERS, MASSACHUSETTS, ASSIGNOR TO BECKWITH MANUFACTURING COMPANY, OF BOSTON, MASSACHUSETTS, A CORPORATION OF MASSACHUSETTS.

## HEEL FOR WOMEN'S SHOES AND METHOD OF MAKING.

Application filed March 7, 1924. Serial No. 697,486.

This invention relates to heels for ladies' shoes made from fibrous material and gums, asphalt or resins. In my application, Serial No. 697,489 filed concurrently herewith is disclosed and claimed a heel or heel base formed by molding under heat and pressure superposed lifts cut from sheet material formed by felting on a paper machine fibrous material having gums, waxes, asphalt, or resins incorporated therewith. When comparatively few lifts are to be employed, as in forming the comparatively low heels or heel bases of men's shoes, this method is entirely satisfactory. When the heels are relatively high, as for women's shoes, the procedure hereinafter outlined is preferable. Since such heels require many lifts and as the cross sectional area of the heel at different elevations varies quite widely, it is desirable to apply pressure thereto in all directions to properly shape the heels and thus avoid the necessity of shaving them after they are fixed to the shoe. The preferred procedure, therefore, is to die out the lifts from the sheet material as it comes wet from the paper machine, allowing in the cutting for shrinkage as the lifts dry out. While wet they are superposed in a heel molding press having its side walls as well as its upper and lower walls relatively movable to press the material. In order that the lifts may be held together paste may be applied to successive lifts as they are placed in the mold or a nail may be driven therethrough substantially centrally thereof. After this preliminary pressing treatment, which acts to expel some of the water and to form the lifts into "biscuits" of general heel shape, the biscuits are allowed to become thoroughly dry. In this form they are in condition to leave the paper mill where the wet sheet or board material from which the lifts were cut was made. Trimmings from the wet fiberboard from which the lifts are cut may be returned directly to the beater engine without any intermediate treatment, hence it is preferable for the biscuits as heretofore described to be made at the paper mill so that the waste from the cutting of the lifts may be salvaged with the minimum trouble and expense.

In order to form the finished heels the dried biscuits are subjected to heat in molds or forms shaped to the desired finished con-

tours, whereupon the gums, asphalt, or resins flux together and unite the lifts in a hard compact mass in the required shape.

For a more complete understanding of this invention, reference may be had to the accompanying drawings in which—

Figure 1 represents a portion of the wet sheet or board from which the lifts are cut.

Figure 2 is a perspective of a biscuit formed by fixing together under pressure superposed lifts cut from the wet board.

Figure 3 is a plan of the mold or die for pressing the lift together.

Figure 4 is a side elevation of the same.

Figure 5 is a section on line 5—5 of Figure 3.

Figure 6 is a view similar to Figure 4, but showing the mold heated for pressing the biscuits into finished heels.

Figure 7 is a front elevation of the finished heel.

Figure 8 is a section on line 8—8 of Figure 7.

The material which may be employed for making the wet sheet material or board from which the lifts are cut is susceptible of wide variation, but as one example, the furnish to be sheeted may be as follows. 60 parts of sulphate pulp, 40 parts of box toe waste, 10 parts of Montan wax, and 4 parts of red oxide, are beaten up together for approximately three hours. 5 parts of silicate of soda may then be added and beaten in for 10 minutes, and 3 parts of alum then added and beaten for 20 minutes, after which the furnish so formed is sheeted into a board of the desired caliper from which the heel lifts will be died out. In place of the sulphate pulp any other cellulose fiber, such as rags, newspaper, or combinations of any cellulose fibers, may be employed. In place of the toe waste, Montan wax may be employed or any waxes, gums, or asphalt or mixtures thereof. In place of the cellulosic materials mentioned leather scrap may be employed. For example, the furnish may comprise 70 parts of leather, 30 parts of toe waste, beaten together hard for 3 hours, 3 parts of silicate of soda beaten in for 10 minutes, 2 parts of resin size beaten in for 10 minutes, and 8 parts of alum beaten in for 20 minutes. Of course any suitable coloring may be employed with any

2  
of the furnishes, red oxide having been hereinbefore indicated in connection with the furnish employing sulphate pulp.

Another furnish which has been found quite satisfactory comprises 50 parts of news; 10 parts of sulphate pulp; 5 parts of Montan wax; 35 parts of toe waste; 8 parts of red oxide, beaten up together, after which 2 parts of rosin size are added and then later 10 3 parts of silicate of soda and then 8 parts of alum or other precipitant.

In each of the furnishes above mentioned, the waxes, gums and resins are fixed to the fibrous material by the rosin size or silicate 15 of soda and the alum so that there is no difficulty in running the stock on the paper machine.

While the sheet is wet the lifts are cut therefrom as indicated in Figure 1, the remaining 20 portions of the sheet as at 2 being then wet and in shape to be broken up and returned directly to the beating engine to be re-incorporated in stock to be sheeted for further use. The lifts cut from the wet 25 material are then placed in a forming mold such as is shown in Figure 3. It will be noted that this mold comprises side sections 3 and a front or breast section 4 which may be relatively moved to press the material 30 therebetween, this movement being effected in the present instance as shown by means of screws 5 threaded through the side walls 6 of the mold and bearing on the outer faces 35 of the members 3 which are slidable in guides 7 in these walls. Preferably the lower face of the mold or die is formed reticulated to permit the escape of water 40 pressed out in the molding operation. Within the upper end of the mold may be inserted a plunger 10 by which the lifts may be compressed together and a proper heel seat form given to the upper surface thereof. This preliminary pressing treatment causes 45 the parts to be united into a somewhat rough heel form of greater size than the finished heel which is then allowed to dry out completely to form the biscuits. These biscuits are then placed in heated molds as shown in Figure 6 similar in construction to that illustrated in Figures 3 to 5 and is then subjected to further pressure and heat. The 50 heat causes the gums, waxes, resins, or asphalt to flux together within the individual lifts and between the lifts to form a hard compact heel whose exterior is so completely finished that no shaving operations are nec-

essary after attachment to the shoe, but only final scouring and polishing operations.

A convenient method of heating the mold is by electric heating units which may be 60 inserted in the pressing elements 3 and in the plunger 10 as shown at 15 in Figure 6. This final molding operation also causes the upper face of the heel to be formed to the required finished concavity without the use 65 of separate rand strips and also causes any size insignia which may be marked on the lower face of the plunger to appear on the heel.

Having thus described this invention it 70 should be evident that many changes and modifications might be made therein without departing from its spirit or scope as defined by the appended claims.

75 I claim:

1. The method of making a heel which comprises pressing together superposed layers of wet fiberboard with thermo-plastic material, drying the biscuit so formed, and molding the dried biscuit to heel form under 80 heat and pressure.

2. The method of making a heel, which comprises fixing together in superposed relation heel lifts cut from wet fiberboard having thermoplastic material therein, molding them under pressure to form biscuits, drying the biscuits so formed, and molding the dried biscuits to heel form under heat and pressure.

3. The method of making a heel which comprises sheeting fibrous material containing thermoplastic material on a paper machine, cutting blanks of the shape of heel lifts from the sheet material while it is still wet, said blanks being large to allow for shrinkage 95 during drying, fixing the wet blanks in superposed relation and subjecting them to pressure to form a biscuit, permitting the biscuit to dry, and molding the dried biscuit to heel form under heat and pressure. 100

4. An unfinished heel or biscuit formed of laminations of felted fibrous material fixed together and containing thermoplastic material.

5. The step product which comprises superposed heel lifts fixed together to form an unfinished heel, each lift comprising felted fibrous material having thermoplastic material incorporated therein.

105 In testimony whereof I have affixed my 110 signature.

ALBERT L. CLAPP.